

## UNITED STATES PATENT OFFICE

2,348,868

PROCESS OF MANUFACTURING FLEXIBLE  
CELLULOSIC PRODUCTSGaston Hubert Vulliet-Durand, Paris, France;  
vested in the Alien Property CustodianNo Drawing. Application March 10, 1939, Serial  
No. 261,154. In France March 19, 1938.

1 Claim. (Cl. 92—21)

The present invention relates to a new plastic sheet material and the process for making the same. The invention is particularly applicable to paper and pasteboard products.

One of the objects of the present invention is to provide a new cellulose pulp product of high flexibility, great strength, and good wearing quality. A further object of the invention is to provide a new use for mannan meal, a by-product of the manufacture of buttons from ivory nuts.

Ordinarily, in the paper and pasteboard industries, it is not possible to use substances which form gelatinous aggregates in the presence of water because such jellylike aggregates prevent proper drainage in the paper machine and obstruct the wire gauze. In the process of the present invention, mannan is used as a gelatinizing substance and the product of the present invention is characterized in that it contains a large proportion of mannan mixed with paper pulp.

According to the present invention, mannan meal is treated with a reagent to alter its properties and to give a product, "insolubilized" mannan, which when mixed with cellulose pulp may be readily formed into sheets. The sheet is then dried and placed in a gelatinizing bath, after which the finished product is dried. The resulting product is flexible and very strong with respect to wear and tear and therefore is capable of extensive use.

The "insolubilized" mannan may be prepared by treatment of mannan meal with a base, alkaline carbonate, lead salt, basic copper or similar reagent prior to its introduction into the cellulose pulp. The invention may be more particularly understood from the following examples:

## Example 1

Mannan meal is placed in a gas tight receptacle and is exposed for a few hours to ammonia gas, after which the excess ammonia is removed by ventilation. The mannan meal thus obtained is transferred to a beater and mixed with water

and cellulose pulp in the proportions of 100 pounds cellulose pulp, 100 pounds insoluble mannan and 56 pounds soluble mannan. The resulting mixture is diluted, and forwarded to either a conventional round or flat table machine and worked up in the usual manner.

## Example 2

Two hundred pounds of mannan meal are heated in a water bath with 45 pounds of potassium or sodium carbonate and sufficient water to dissolve the carbonate, after which a precipitation agent for the pseudosolution of mannan is added. Any precipitation or jellification agent of the pseudosolution of mannan can be employed as for example, alcohol or acetone. The whole mixture is then transferred to a centrifugal drying machine and after washing the treated mannan is transferred to a beater and mixed with cellulose pulp as in Example 1. The product thus obtained is converted on a paper machine to sheets or other shapes and dried in known manner by a press or a centrifugal machine, after which it is kept in a bath for gelatinizing the mannan. Satisfactory results may be obtained by using acidulated water, aqueous glycerine, or formaldehyde in the gelatinizing bath. The finished plastic sheet is obtained after a final drying.

The foregoing description has been given by way of example only and the details may be varied without departing from the principle and scope of the invention.

Having thus described my invention, what I claim is:

The process for the production of a flexible cellulose pulp product which comprises solubilizing mannan by heating with a solution of sodium carbonate, precipitating the mannan with alcohol, mixing the precipitated mannan with cellulose pulp, giving the mixture the desired form, drying the formed material, soaking the form in a bath of acidulated water and finally drying.

GASTON HUBERT VULLIET-DURAND.